

## 1

3,189,547

## LUBRICATING COMPOSITIONS

George M. Calhoun, Berkeley, Calif., assignor to Shell Oil Company, a corporation of Delaware  
No Drawing. Filed July 3, 1959, Ser. No. 824,796  
8 Claims. (Cl. 252—48.6)

This invention relates to lubricants, particularly those useful for lubrication under severe operating conditions, such as those under extreme high speed and at high temperatures and to a new and novel class of compounds therefor.

It is well known that the high pressure occurring in certain types of gears and bearings may cause rupture of lubricant films with consequent damage to the machinery. It is known that various base lubricants can be improved in their protective properties for rubbing surfaces by the addition of certain substances, so-called extreme pressure agents, so that excessive wear, scuffing and seizure which normally follow a break in the film lubricant are minimized or prevented.

It is known that certain compounds of metal-reactive elements, such as certain compounds of chlorine, sulfur and phosphorus, as well as certain other compounds, such as some compounds of lead, impart extreme pressure properties to various lubricants. Notable among the substances heretofore used are the lead soaps, phosphoric acid esters, free or bound sulfur and certain chlorinated organic compounds. A principal objection to many of these extreme pressure agents is their generally high reactivity with the metallic surface, causing etching, corrosion and discoloration of the metal surface. Another objection to chemically reactive extreme pressure agents is that they alter the original chemical nature of the contacting surface, which under certain conditions is undesirable. Additionally, because of the activity of agents of this type, they usually are depleted rapidly resulting in only a temporary solution to the problem of extreme pressure lubrication.

It has now been discovered that improved extreme pressure lubricants are provided by a suitable lubricating oil containing an oil-soluble polythioether-ester-ether derivative obtained by reacting (a) an ester of a long chain unsaturated fatty acid, RCOOH, and a polyoxyalkylene diol or its thio derivative having the formula



where R' and R'' are the same or different alkyl radicals of from 2 to 8, preferably 2 to 3 carbon atoms, X is oxygen or sulfur and x and y are integers of at least 1, preferably 1 to 6 with (b) a mercapto compound such as a mercapto acid, alcohol, ether or ester so that the end product has at least 1 and preferably 2 thioether radicals



where Z is —OR''' or —COOR''' and the R''' is hydrogen or a C<sub>1-4</sub> alkyl radical and n is an integer of from 1 to 4, preferably 1. The maximum number of



units in the final compound depends on the degree of unsaturation of the intermediate ether-ester. The unsat-

## 2

urated fatty acid ester of the polyoxyalkylene glycol may be represented by the corresponding formula



and the thioether thereof by the formula



The intermediate ether-esters are prepared by esterifying a long chain unsaturated fatty acid such as oleic acid, linoleic acid, linolenic acid, erucic acid, ricinoleic acid and the like with a polyoxyalkylene diol or the thio derivatives thereof, such as diethylene glycol, triethylene glycol, tetraethylene glycol, dipropylene glycol, tripropylene glycol, dibutylene glycol, 2,2'-thiodiethanol, 3,3'-thiodipropanol, and the like. Esters of these materials include diethylene glycol dioleate, triethylene dioleate, dipropylene glycol dioleate, diethylene glycol linoleate, tetraethylene glycol ricinoleate, dibutylene glycol oleate, 2,2'-thiodiethanol dioleate, 2,2'-thiodiethanol diricinoleate, 2,2'-thiodiethanol linoleate and the like.

Compounds of the present invention are prepared by reacting the ether-ester with a mercapto compound such as mercapto aliphatic carboxylic acids, e.g., mercaptoacetic acid, mercaptopropionic acid, mercaptobutyric acid, or mercapto-alkanols such as 2-mercaptoethanol, 2- and 3-mercaptopropanol, 2-, 3- and 4-mercaptopbutanol or ethers of said mercaptoalcohols such as methyl or octyl 2-mercaptopethanol or mercapto esters, e.g., ethyl mercaptoacetate or ethyl mercaptobutyrate, and mixtures thereof.

The additives can be prepared by the methods described by Koenig et al., JACS, 79, 362 (1957), or Fitzgerald, Jr., Org. Chem., 22, 197 (1957), and preferably at low temperatures, from room temperature to about 50° C., in the presence of a free radical catalyst such as azo or peroxide catalysts or ultraviolet light and a non-reactive solvent such as benzene, toluene, xylene, or the like. Suitable initiators include various free radical-yielding, heterocyclic and alicyclic peroxides, such as diethyl peroxide, tertiary butyl hydroperoxide, dibenzoyl peroxide, di-tert-butyl peroxide, dimethylthienyl peroxide, dicyclohexyl peroxide, dilauroyl peroxide and urea peroxide. These are mentioned by way of non-limiting examples of suitable organic peroxides. Other initiating compounds known include emulsion redox systems, such as a mixture of sodium bisulfite and persulfate, ammonium persulfate, alkali metal perborates azo compounds, such as alpha, alpha-azodiisobutyronitrile, etc.

The following examples illustrate the preparation of suitable additives for use in accordance with the present invention.

## EXAMPLE I

About 600 grams of diethylene glycol dioleate and 223.5 grams of mercaptoacetic acid were mixed in a flask at 20-25° C. About 240 drops (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over Na<sub>2</sub>SO<sub>4</sub>, filtered and the solvent stripped at 155° C. and 2 mm. pressure. The final product was a mixture of the 9- and the 10-carboxymethylmercaptostearate diesters of diethylene glycol.

3  
EXAMPLE II

About 600 grams of triethylene glycol dioleate and 223.5 grams of mercaptoacetic acid were mixed in a flask at 20-25° C. About 240 (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 2 mm. pressure. The final product was a mixture of the 9- and 10-carboxymethylmercaptostearate diesters of triethylene glycol.

EXAMPLE III

About 600 grams of diethylene glycol in ricinoleate and 223.5 grams of mercaptoacetic acid were mixed in a flask of 20-25° C. About 240 drops (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 2 mm. pressure. The final product was a mixture of the 9- and 10-carboxymethylmercaptostearate diesters of diethylene glycol.

EXAMPLE IV

About 600 grams of diethylene glycol dioleate and 223.5 grams of mercaptoethanol were mixed in a flask at 20-25° C. About 240 drops (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 12 mm. pressure. The final product was a mixture of diethylene glycol di(9- and 10-[2-hydroxyethylmercapto]stearate).

EXAMPLE V

About 600 grams of 2,2'-thiodiethanol dioleate and 223.5 grams of mercaptoacetic acid were mixed in a flask at 20-25° C. About 240 drops (30 drops at a time) of t-butyl hydroperoxide were added over a period of 2 hours and the temperature was kept at about 37° C. The reaction mixture was diluted with 2 volumes of diethyl ether, washed with 12 liters of water to pH 4, dried over  $\text{Na}_2\text{SO}_4$ , filtered and the solvent stripped at 155° C. and 2 mm pressure. The final product was a mixture of 2,2'-thiodiethanol di(9- and 10-carboxymethylmercaptostearate).

The mercapto-modified polyether-esters are oil-soluble and can be used in amounts of from about 0.5% to about 20%, preferably from about 1% to about 5% by weight.

Lubricating oils useful for the preparation of compositions of this invention can be one or more of a variety of synthetic oils or natural hydrocarbon oils having a viscosity range of from 50 SUS at 100° F. to 250 SUS at 210° F.—(SAE viscosity number ranging from SAE 10W to SAE 90). The natural hydrocarbon oils can be obtained from paraffinic naphthenic, asphaltic or mixed base crudes, and/or mixtures thereof refined as by extraction, acid treatment, clay treatment. Synthetic oils include polymerized olefins, alkylated aromatics, isomerized waxes, copolymers of alkylene glycols and alkylene oxide (Ucon fluids) which are described in U.S. Patents 2,425,755, 2,425,845 and 2,774,733 such as Ucon 50HB170, Ucon 50HB660 or Ucon LB550X and which are copolymers of ethylene and 1,2-propylene oxides, the mono- and diols, as well as their ether derivatives; organic esters of aliphatic dibasic acids such as di-2-ethylhexyl sebacate or di-2-ethylhexyl adipate and the like. The hydrocarbon oils may be blended with fixed oils such as castor oil, lard oil and the like and/or synthetic oils as mentioned or silicone polymers and the like. Typical oils of this type include petroleum motor

oils which are (A) paraffinic in character and (B) naphthenic in character having the following properties:

|                           | (A) (SAE 10W) | (B) (SAE 30) |
|---------------------------|---------------|--------------|
| 5                         |               |              |
| Pour point, ° F.          | -10           | -5           |
| Flash, ° F.               | 390           | 415          |
| Viscosity, SUS at 210° F. | 44            | 58           |
| Viscosity index           | 90            | 60           |

10 Other suitable oils are the gas turbine lube oils having the following properties:

|                           | Grade | 1010 | 1065 |
|---------------------------|-------|------|------|
| 15                        |       |      |      |
| Flash, COC, ° F.          | 300   | 465  |      |
| Pour, ° F.                | -10   | 0    |      |
| Viscosity, SUS at 100° F. | 59.4  | 530  |      |
| Neutral Number            | 0.02  | 0.01 |      |
| Ash                       | None  | None |      |

20 The following compositions are illustrative of the invention, the percentages being by weight:

*Composition A*

25 Example I additive ----- 2%.  
1010 mineral oil ----- Essentially balance.

*Composition B*

Example II additive ----- 2%.  
30 1010 mineral oil ----- Essentially balance.

*Composition C*

Example III additive ----- 2%.  
1010 mineral oil ----- Essentially balance.

*Composition D*

Example IV additive ----- 2%.  
1010 mineral oil ----- Essentially balance.

*Composition E*

40 Example II additive ----- 1%.  
SAE 30 mineral oil ----- Essentially balance.

*Composition F*

Example V additive ----- 2%.  
45 SAE 90 mineral oil ----- Essentially balance.

*Composition G*

Example I additive ----- 2%.  
Lauric acid ----- 2%.  
50 SAE 90 mineral oil ----- Essentially balance.

*Composition H*

Example I additive ----- 5%.  
Ucon 50HB660 (polyethylene-propylene glycol having a SUS at 100° F. of 660) ----- Essentially balance.

*Composition I*

60 Example I additive ----- 2%.  
Di-2-ethylhexyl sebacate ----- Essentially balance.

Compositions of this invention were evaluated for their extreme pressure properties on a spur-gear machine. The machine consists essentially of two geometrically similar pairs of gears connected by two parallel shafts. The gear pairs are placed in separate gear boxes, which also contain the supporting ball bearings. One of the shafts consists of two sections connected by a coupling. Loading is accomplished by locking one side of the coupling and applying torque to the other. The conditions of the test were:

Speed ----- r.p.m. 3200

Oil temperature ----- ° C. 100

Oil flow-rate ----- cc./sec. 10

70 75 Load in increments 5 min. at each setting.

Results of the evaluations are given in Table I and for purpose of comparison, the results obtained from the use of the base oil alone and with other known extreme pressure compositions are also given.

TABLE I

| Composition:                                                           | Score load, lbs./in.  |
|------------------------------------------------------------------------|-----------------------|
| A, B, C and E through I                                                | 10,000-12,000.        |
| 1010 mineral oil+2% C <sub>16</sub> alkenyl succinic acid              | 1,400 (3,200 r.p.m.). |
| 1010 mineral oil+2% maleic acid                                        | 2,800.                |
| 1010 mineral oil+2% 3-hexadecyl adipic acid                            | 1,400.                |
| 1010 mineral oil+2% dodecyl-mercaptopsuccinic acid                     | 1,400.                |
| 1010 mineral oil+10% glycerol monooleate                               | 1,800.                |
| 1010 mineral oil+2% C <sub>13</sub> H <sub>27</sub> OH ("OXO" process) | 600.                  |
| 1010 mineral oil                                                       | 600.                  |

The data show the outstanding enhancement of the load-carrying ability of the oil effected by the mercapto-containing compounds of the invention, as represented by those of Compositions A through I. On the other hand, malonic acid, succinic acid, 3-hexadecyl adipic acid and C<sub>16</sub>-alkenyl succinic acid as well as sulfur-containing acids outside the scope used by applicant such as dodecyl-mercaptop-succinic acid, or other types of esters and alcohols such as glycerol-monooleate, lauric acid or "OXO" alcohol effected only a slight improvement.

Compositions of the present invention were also tested for their corrosion and sludge resistant properties by the following methods: (1) a Timken 2126 steel bearing was immersed in a test composition and placed in an open air over at 150° C. for 65 hours, and at the end of the test, the bearing examined and (2) steel rods (3/16" by 3") were immersed in test compositions for 21½ hours at 150° C. and the amount of sludge formed on the rods was noted as shown in Table II.

TABLE II

| Composition                                          | 1             | 2               |
|------------------------------------------------------|---------------|-----------------|
| Composition A                                        | No stain      | 0.7 mg. sludge. |
| 1010 Mineral oil + 2% 3-(2-ethylhexyl)adipic acid.   | Badly stained | 60 mg. sludge.  |
| 1010 Mineral oil + 2% 9- and 10-carboxystearic acid. |               | 100 mg. sludge. |

The sulfur-containing compounds of this invention are useful also for providing superior load-carrying properties for lubricating oils which contain minor amounts of other agents, such as silicone anti-forming agents, alkyl-phenol anti-oxidants, polyacrylate ester viscosity-index improvers, long chain acids such as lauric and oleic acids as oiliness agents and the like.

I claim as my invention:

1. A mineral lubricating oil composition comprising a major amount of mineral lubricating oil and from about 0.5% to about 20% of an oil-soluble dithiaether derivative of a diester of a long chain unsaturated fatty acid

having 18 carbon atoms and a diol selected from the group consisting of polyethylene glycol and 2,2'-thiodiethanol, the thioether radical components of the ester being represented by



where Z is a polar radical selected from the group represented by —OR'' and —COOR'' and R'' is selected from the group consisting of hydrogen and C<sub>1-4</sub> alkyl radical and n is an integer of from 1 to 4.

2. A mineral lubricating oil composition comprising a major amount of mineral lubricating oil and from about 1% to about 5% of an oil-soluble dicarboxy C<sub>1-4</sub> alkyl mercapto stearate diester of polyethylene glycol.

3. A mineral lubricating oil composition comprising a major amount of mineral lubricating oil and from about 1% to about 5% of an oil-soluble dicarboxy C<sub>1-4</sub> alkyl mercapto hydroxystearate diester of polyethylene glycol.

4. A mineral lubricating oil composition comprising a major amount of mineral lubricating oil and from about 1% to about 5% of di(carboxy-C<sub>1-4</sub> alkyl mercapto) containing 2,2'-thiodiethanol dioleate.

5. A mineral lubricating oil composition comprising a major amount of mineral lubricating oil and from about 1% to about 5% of dicarboxymethylmercapto stearate diester of diethylene glycol.

6. A mineral lubricating oil composition comprising a major amount of mineral lubricating oil and from about 1% to about 5% of di(carboxymethylmercapto) containing 2,2'-thiodiethanol dioleate.

7. A mineral lubricating oil composition comprising a major amount of mineral lubricating oil and from about 1% to about 5% of a mixture of 9- and 10-carboxymethylmercapto stearate diester of diethylene glycol.

8. A mineral lubricating oil composition comprising a major amount of mineral lubricating oil and from about 1% to about 5% 2,2'-thiodiethanol di(9- and 10-carboxymethylmercapto stearate).

#### References Cited by the Examiner

#### UNITED STATES PATENTS

|    |           |       |                  |            |
|----|-----------|-------|------------------|------------|
| 45 | 2,073,841 | 3/37  | Humphreys et al. | 252-48.6   |
|    | 2,318,629 | 5/43  | Pruton           | 252-48.6 X |
|    | 2,454,568 | 11/48 | Pollock          | 260-399    |
|    | 2,476,129 | 7/49  | Augustine        | 260-399    |
| 50 | 2,540,570 | 2/51  | Cyphers          | 252-48.6   |
|    | 2,649,416 | 8/53  | Richter et al.   | 252-48.6   |
|    | 2,994,662 | 8/61  | Calhoun et al.   | 252-48.6   |
|    | 3,041,283 | 6/62  | Calhoun et al.   | 252-48.6   |
|    | 3,041,284 | 6/62  | Calhoun et al.   | 252-48.6   |

#### FOREIGN PATENTS

|    |         |       |                |
|----|---------|-------|----------------|
| 55 | 520,034 | 12/55 | Canada.        |
|    | 657,750 | 9/51  | Great Britain. |

DANIEL E. WYMAN, Primary Examiner.

60 JULIUS GREENWALD, JOSEPH R. LIBERMAN,  
Examiners.